

# United States Patent [19]

Kozlowski et al.

[11] 3,901,664

[45] Aug. 26, 1975

[54] MOTOR FUEL

[75] Inventors: **Robert H. Kozlowski**, Berkeley; **Joel W. Rosenthal**, El Cerrito, both of Calif.

[73] Assignee: **Chevron Research Company**, San Francisco, Calif.

[22] Filed: **Nov. 23, 1973**

[21] Appl. No.: **418,522**

**Related U.S. Application Data**

[63] Continuation of Ser. No. 163,513, June 25, 1971, abandoned.

[52] U.S. Cl. .... **44/56**; 260/632 C

[51] Int. Cl.<sup>2</sup> .... **C10L 1/08**

[58] Field of Search .... **44/56; 208/16, 17**

[56] **References Cited**

UNITED STATES PATENTS

|           |         |                   |        |
|-----------|---------|-------------------|--------|
| 1,516,907 | 11/1924 | Backhaus.....     | 44/56  |
| 1,757,837 | 5/1930  | Johns.....        | 44/56  |
| 1,757,838 | 5/1930  | Johns.....        | 44/56  |
| 1,907,309 | 5/1933  | Schaack, Jr.....  | 44/56  |
| 2,087,582 | 7/1937  | Schneider.....    | 44/56  |
| 2,852,356 | 9/1958  | Lichtenfels.....  | 208/17 |
| 2,897,067 | 7/1959  | Sparks et al..... | 44/56  |
| 3,172,834 | 3/1965  | Kozlowski.....    | 208/17 |

3,455,664 7/1969 Rosscup et al..... 44/56  
3,576,891 4/1971 Rosenthal ..... 44/56

Primary Examiner—Daniel E. Wyman

Assistant Examiner—Mrs. Y. H. Smith

Attorney, Agent, or Firm—G. F. Magdeburger; R. H. Davies; J. J. De Young

[57] **ABSTRACT**

A motor fuel comprising 1–40 volume percent oxylate and 99–60 volume percent light hydrocrackate.

The oxylate consists of tertiary butyl alcohol, isopropyl alcohol, and methyl alcohol. Preferred composition for the oxylate is about 20–90 volume percent tertiary butyl alcohol, 5–40 volume percent isopropyl alcohol, and 5–40 volume percent methyl alcohol.

The light hydrocrackate preferably boils between about pentane and 250°F. as opposed to full-boiling-range gasoline, which would boil up to about 430°F. The oxylate improves the octane of the light hydrocrackate gasoline more than expected, and also the oxylate has an unexpectedly high blending octane number in the light hydrocrackate over a wide range of percentage amounts of oxylate in the light hydrocrackate.

**7 Claims, No Drawings**

## MOTOR FUEL

This is a continuation of application Ser. No. 163,513, filed June 25, 1971, now abandoned.

## BACKGROUND OF THE INVENTION

The present invention relates to a motor fuel composition comprising hydrocarbons and alcohols. The motor fuel is particularly intended for use in automobiles, but can be used in other engines such as boat engines and aircraft engines. The motor fuel composition of the present invention comprises gasoline which, as is well known, is essentially a hydrocarbon mixture having suitable volatility for operating internal combustion engines with spark ignition. The motor fuel composition can contain other additives such as oiliness agents, gum solvents, dyes, gum inhibitors, antioxidants, rust preventatives, and the like. The motor fuel can also contain lead additives. However, one of the advantages of the composition of the present invention is that it provides a relatively high-octane gasoline without the use of lead additives, or with the use of only a relatively small amount (e.g., 1.5 cc. alkyl lead additive or less per gallon of motor fuel) of lead additive.

The use of alcohols in gasoline-boiling-range hydrocarbons has been suggested in a number of patents.

For example, U.S. Pat. No. 1,839,362 and U.S. Pat. No. 2,596,198 suggest the use of methyl alcohol in gasoline.

U.S. Pat. No. 2,662,817 and U.S. Pat. No. 2,726,942 disclose the use of methyl alcohol and isopropyl alcohol in gasoline.

U.S. Pat. No. 2,850,368 discloses the use of isopropyl alcohol and secondary butyl alcohol in gasoline. U.S. Pat. No. 2,197,378 discloses the use of isopropyl alcohol and n-butyl alcohol in gasoline.

U.S. Pat. Nos. 2,365,009, 2,404,094 and 2,408,999 all disclose the use of methyl alcohol, isopropyl alcohol, and tertiary butyl alcohol, amongst a wide range of other possible alcohols, for use in gasoline. The latter three patents are directed to major amounts of alcohol containing a minor or small amount of hydrocarbon component; for example, 95 to 90 volume percent alcohol component with only 5 to 10 volume percent hydrocarbon component.

In addition to the above patents concerned primarily with alcohol-gasoline compositions, there are a number of patents directed to other additives for gasoline. For example, U.S. Pat. No. 3,083,087 is directed to use of benzyl esters in gasoline; U.S. Pat. No. 2,874,033 is directed to the use of isopropyl ether plus isopropyl alcohol in gasoline; and U.S. Pat. No. 1,399,227 is directed to the use of acetone in gasoline.

## SUMMARY OF THE INVENTION

The composition of matter of the present invention is a motor fuel comprising 1-40 volume percent oxylate and 99-60 volume percent light hydrocrackate.

The term "oxylate" is used to mean a mixture of tertiary butyl alcohol, isopropyl alcohol, and methyl alcohol.

Table I lists composition ranges for the oxylate.

The present invention is based upon a number of features. The following features of the present invention can be mentioned.

We have found that the oxylate gives an unexpectedly high blending octane number in light hydrocrackate, particularly when compared to the blending octane number for the oxylate in full-boiling-range gasoline stocks; that is, gasoline stocks which tend to boil over a wider boiling range than does light hydrocrackate. Light hydrocrackate, which is used in the composition according to the present invention, usually boils between about pentane and 250°F. Preferably about 90 volume percent of the light hydrocrackate boils below about 200°F. More preferably, at least 90 volume percent of the light hydrocrackate boils between pentane and 180°F. Full-boiling-range gasoline stocks usually boil between about butane and 430°F.; and the 90 volume percent point for full-boiling-range gasoline stocks is generally considerably above 250°F., for example about 340°F.

For about 5-40 percent oxylate in light hydrocrackate, we have found the blending octane number to be about 120, contrasted to a blending octane number of about 110 for oxylate in full-boiling-range gasoline stocks. This unexpected incremental amount for the blending octane number of oxylate in light hydrocrackate compared to oxylate in full-boiling-range gasoline stocks is not expected; thus, oxylate plus light hydrocrackate is a synergistic combination.

In addition to the synergistic result obtained by adding the oxylate composition to the gasoline in accordance with the present invention, a second feature of the present invention is that the oxylate is of sufficiently high octane number that it can be used to substantially increase the octane number of light hydrocrackate in much the same way that lead additives and/or aromatics are used. Thus, oxylate can be used to reduce the concentration of lead additives and/or aromatics in light hydrocrackate without sacrificing octane number.

A third particular feature of the present invention which can be mentioned is that the oxylate composition used has a relatively high solubility in light hydrocrackate and is not extracted from light hydrocrackate easily as is methanol or ethanol.

Furthermore, an additional (fourth) feature of the composition of the present invention is the integration of the light hydrocrackate production step with the oxylate production step. The hydrocracking process used to produce the light hydrocrackate produces substantial quantities of isobutane, and it is particularly preferred in producing the composition of the present invention to use at least a portion of the isobutane from the hydrocracking step as at least a portion and preferably as all of the isobutane feedstock to the isobutane oxidation step for the production of oxylate. According to a preferred embodiment of the present invention, the isobutane which is oxidized is produced in the hy-

TABLE I

| Component         | Broad Range, Volume % | Preferred Range, Volume % | Most Preferred Range, Vol. % |
|-------------------|-----------------------|---------------------------|------------------------------|
| t-Butyl alcohol   | 2-90                  | 20-90                     | 40-60                        |
| Isopropyl alcohol | 2-50                  | 5-40                      | 20-30                        |
| Methyl alcohol    | 2-50                  | 5-40                      | 20-30                        |

drocracking step of an "all-hydrocracking" refinery, for example, in a refinery process such as described in U.S. Pat. No. 3,537,977.

A particularly preferred process embodiment for producing a gasoline composition in accordance with the present invention (and also having essentially no aromatics, i.e., less than 2 volume percent aromatics) is as follows. A C<sub>5</sub>+ hydrocarbon fraction is fed to a fractionation zone and split into at least a C<sub>5</sub>-C<sub>6</sub> fraction and a C<sub>7</sub>+ fraction. The C<sub>5</sub>-C<sub>6</sub> fraction is isomerized to produce a relatively high-octane (80-90 research octane number) product. The C<sub>7</sub>+ fraction is fed to a hydrocracking zone wherein the C<sub>7</sub>+ feed is hydrocracked to produce a product including light hydrocrackate and isobutane. Effluent from the hydrocracking zone is separated into a propane and lighter fraction, an isobutane fraction, a C<sub>5</sub>-C<sub>6</sub> or approximately light hydrocrackate-boiling-range fraction, and a C<sub>7</sub>+ fraction. The isobutane is subjected to sequential oxidation and hydrogenation to produce oxylate alcohols having a high octane number (BON, about 110 or more). The C<sub>7</sub>+ fraction or at least a large portion of the C<sub>7</sub>+ fraction is recycled to the hydrocracking zone to enable large production of isobutane and light hydrocrackate from the hydrocracking step. The light hydrocrackate is blended with alcohols and preferably with the isomerization zone product to produce a high-octane, essentially aromatic-free, low-end-point unleaded gasoline.

The term "hydrocracking" is used in the present specification to mean a catalytic process carried out at a temperature between about 500° and 900°F. for the conversion of a hydrocarbon feedstock to more valuable hydrocarbons, particularly including gasoline, by contacting the hydrocarbon feedstock with a hydrocracking catalyst in the presence of hydrogen gas.

The hydrocracking catalysts used in hydrocracking typically are Group VI or Group VIII metal components with an inorganic refractory carrier such as alumina and/or silica. Catalytic hydrocracking is a well-known process and is described, for example, in HYDROCARBON PROCESSES, September, 1968, pages 139-144.

A fifth feature of the present invention, which is very important is that we have devised a particularly advantageous process for manufacturing the oxylate for use in gasoline. Instead of starting with feedstocks such as olefins to obtain alcohols, we start with isobutane feedstock, which is present in many refineries in excess amounts, particularly refineries wherein hydrocracking is carried out to produce gasoline-boiling-range hydrocarbons. In our preferred process the isobutane is oxidized to form tertiary butyl alcohol and acetone plus small amounts of methanol and esters. This process is described in more detail in our concurrently filed application entitled "GASOLINE PRODUCTION" (attorney's docket No. B-1812A), the disclosure of which application is incorporated by reference into the present application. The effluent from the oxidation step is hydrogenated to obtain an oxylate mixture comprising t-butyl alcohol, isopropyl alcohol, and methyl alcohol.

Thus, with respect to this fifth feature, it can be said in summary that we have devised and developed a process to make large amounts of oxylates in a refinery at relatively low cost for use in a gasoline composition.

5 Table II below tabulates data comparing the blending octane number (BON) of oxylate in light hydrocrackate to the blending octane number of oxylate in full-boiling-range gasoline.

TABLE II

|    |           | BON for<br>Oxylate-Light<br>Hydrocrackate <sup>1</sup> | BON<br>for Oxylate<br>in Full<br>Boiling Range<br>Gasoline <sup>2</sup> |
|----|-----------|--------------------------------------------------------|-------------------------------------------------------------------------|
| 10 |           |                                                        |                                                                         |
| 15 | % Oxylate | 10 122<br>20 120<br>40 120                             | 110<br>105<br>100                                                       |

<sup>1</sup>90% pt. (ASTM D-86) 212; RON 81.5

<sup>2</sup>90% pt. (ASTM D-86) 338; RON 89.5

20 To obtain the data for Table II, mixtures of base gases and oxylate were prepared and the research octane numbers (RON) (unleaded) of the bases and the mixtures determined. The BON's were calculated with the following formula:

25

$$BON_{oxylate} = \frac{O_F - X_B(O_B)}{X_{oxylate}}$$

30

X<sub>B</sub> = Vol. Fract. of base

O<sub>B</sub> = Octane of base

X<sub>oxylate</sub> = Vol. Fract. of oxylate

O<sub>F</sub> = RON of Blend

35

Although various embodiments of the invention have been described, it is to be understood that they are meant to be illustrative only and not limiting. Certain features may be changed without departing from the spirit or scope of the present invention. It is apparent that the present invention has broad application to motor fuel compositions containing oxylate in light hydrocrackate. Accordingly, the invention is not to be construed as limited to the specific embodiments or examples discussed, but only as defined in the appended claims or substantial equivalents of the claims.

40

What is claimed is:

45

1. A motor fuel comprising 1-40 volume percent oxylate and 99-60 volume percent light hydrocrackate, said hydrocrackate containing essentially no aromatics, and said oxylate being a mixture of t-butyl alcohol, isopropyl alcohol and methyl alcohol and containing an amount, based upon 100 volumes of said oxylate, of t-butyl alcohol in the range 2-90 volumes, of isopropyl alcohol in the range 2-50 volumes, and of methyl alcohol in the range 2-50 volumes.

50

2. A motor fuel in accordance with claim 1 wherein the oxylate contains 20-90 volume percent t-butyl alcohol, 5-40 volume percent isopropyl alcohol, and 5-40 volume percent methyl alcohol.

55

3. A motor fuel in accordance with claim 1 wherein the oxylate contains about 40-60 volume percent t-butyl alcohol, about 20-30 volume percent isopropyl alcohol, and about 20-30 percent methyl alcohol.

60

4. A motor fuel in accordance with claim 1 wherein at least about 90 volume percent of the light hydrocrackate boils below 200°F.

65

5. A motor fuel in accordance with claim 1 wherein at least 90 volume percent of the light hydrocrackate boils between about pentane and 180°F.

6. A motor fuel in accordance with claim 1 wherein the oxylate is prepared at least in part by a process which comprises oxidizing isobutane to obtain t-butyl alcohol, acetone, and methyl alcohol, and then hydrogenating the effluent from the oxidation step to obtain a mixture comprising t-butyl alcohol, isopropyl alcohol, and methyl alcohol.

7. A process in accordance with claim 5 wherein the motor fuel is prepared at least in part by blending light hydrocrackate from a hydrocracking process with the oxylate, and wherein the oxylate is prepared at least in part by the oxidation of isobutane from said hydrocracking process.

\* \* \* \* \*

10

15

20

25

30

35

40

45

50

55

60

65